# EUROPEAN PATENT SPECIFICATION

(11) **EP 1 244 548 B1**
(45) Date of publication and mention of the grant of the patent: **16.06.2004**
(21) Application number: 00982378.2
(22) Date of filing: 04.12.2000
(51) Int. Cl.: B41C 1/10, B41M 5/36

(54) **HEAT-SENSITIVE IMAGING ELEMENT FOR PROVIDING LITHOGRAPHIC PRINTING PLATES**
WÄRMEEMPFINDLICHES BILDAUFZEICHNUNGSELEMENT ZUR HERSTELLUNG LITHOGRAPHISCHER DRUCKPLATTEN
ELEMENT THERMOSENSIBLE POUR PREPARER UNE PLAQUE D'IMPRESSION LITHOGRAPHIQUE

(30) Priority: 03.12.1999 US 454151; 23.08.2000 US 644600
(43) Date of publication of application: 02.10.2002
(62) Divisional of application: 03028448.3
(73) Proprietor: Kodak Polychrome Graphics Company Ltd., Norwalk, Connecticut 06851 (US)
(72) Inventor: LEON, Jeffrey, W., Rochester, NY 14650 (US); FLEMING, James, C., Webster, NY 14580 (US)
(74) Representative: Pidgeon, Robert John
(86) International application number: PCT/US2000/032841
(87) International publication number: WO 2001/039985

(56) References cited:
- EP-A- 0 980 754
- EP-A- 1 031 412
- US-A- 5 910 395

## Description

### FIELD OF THE INVENTION

This invention relates in general to lithographic printing plates and specifically to lithographic printing plates that require no wet processing after imaging. The invention also relates to a method of digitally imaging such imaging members, and to a method of printing using them.

### BACKGROUND OF THE INVENTION

The art of lithographic printing is based upon the immiscibility of oil and water, wherein an oily material or ink is preferentially retained by an imaged area and the water or fountain solution is preferentially retained by the non-imaged areas. When a suitably prepared negative working printing plate is moistened with water and ink is then applied the background or non-imaged areas retain the water and repel the ink while the imaged areas accept the ink and repel the water. The reverse holds true for positive working plates, in which the background is imaged. The ink is then transferred to the surface of a suitable substrate, such as cloth, paper or metal, thereby reproducing the image.

Very common lithographic printing plates include a metal or polymer support having thereon an imaging layer sensitive to visible or UV light. Both positive and negative-working printing plates can be prepared in this fashion. Upon exposure, and perhaps post-exposure heating, either imaged or non-imaged areas are removed using wet processing chemistries.

Thermally sensitive printing plates are less common, yet represent a steadily growing market. Currently, most of these plates utilize similar materials and similar imaging mechanisms as UV-imageable plates. For example, a thermal acid generator might be used in lieu of a photoacid generator and the same series of preheat and development steps might be employed. The main advantage of these digital plates is that the thermal imaging process is rapid and inexpensive compared to the analog process involving the creation of a mask and blanket UV exposure. Examples of such plates are described in US-A-5,372,915 (Haley et al.). They include an imaging layer comprising a mixture of dissolvable polymers and an infrared radiation absorbing compound. While these plates can be imaged using lasers and digital information, they require wet processing using alkaline developer solutions.

It has been recognized that a lithographic printing plate could be created by ablating an IR absorbing layer. For example, Canadian 1,050,805 (Eames) discloses a dry planographic printing plate comprising an ink receptive substrate, an overlying silicone rubber layer, and an interposed layer comprised of laser energy absorbing particles (such as carbon particles) in a self-oxidizing binder (such as nitrocellulose). Such plates were exposed to focused near IR radiation with a Nd⁺⁺YAG laser. The absorbing layer converted the infrared energy to heat thus partially loosening, vaporizing or ablating the absorber layer and the overlying silicone rubber. The plate was developed by applying naphtha solvent to remove debris from the exposed image areas. Similar plates are described in *Research Disclosure* 19201, 1980 as having vacuum-evaporated metal layers to absorb laser radiation in order to facilitate the removal of a silicone rubber overcoated layer. These plates were developed by wetting with hexane and rubbing. CO, lasers are described for ablation of silicone layers by Nechiporenko & Markova, PrePrint 15th International IARIGAI Conference, June 1979, Lillehammer, Norway, Pira Abstract 02-79-02834. Typically, such printing plates require at least two layers on a support, one or more being formed of ablatable materials. Other publications describing ablatable printing plates include US-A-5,385,092 (Lewis et al.), US-A-5,339,737 (Lewis et al.), US-A-5,353,705 (Lewis et al.), US Reissue 35,512 (Nowak et al.) and US-A-5,378,580 (Leenders).

While the noted printing plates used for digital, processless printing have a number of advantages over the more conventional photosensitive printing plates, there are a number of disadvantages with their use. The process of ablation creates debris and vaporized materials that must be collected. The laser power required for ablation can be considerably high, and the components of such printing plates may be expensive, difficult to coat, or unacceptable in resulting printing quality. Such plates generally require at least two coated layers on a support.

One approach toward non-process, non-ablation printing plates involves the use of "switchable polymers." These polymers will undergo thermally driven chemical reactions in which highly polar moieties are either created or destroyed under imaging conditions. This results in the storage of the imaging data as hydrophilic and hydrophobic regions of a continuous polymer surface. In addition to being not needing wet processing, such plates have the advantage of not needing any type of material collection devices which ablation-based plates require. Also unlike ablation plates, a switchable polymer plate in its ideal form would consist of one layer and can be manufactured on a single pass through a coating machine.

US-A-4,034,183 (Uhlig) describes the use of high powered lasers to convert hydrophilic surface layers to hydrophobic surfaces. A similar process is described for converting polyamic acids into polyamides in US-A-4,081,572 (Pacansky). The use of high-powered lasers is undesirable in the industry because of their power requirements and because of their need for cooling and frequent maintenance.

US-A-4,634,659 (Esumi et al.) describes imagewise irradiating hydrophobic polymer coatings to render exposed regions more hydrophilic in nature. While this concept was one of the early applications of converting surface characteristics in printing plates, it has the disadvantages of requiring long UV light exposure times (up to 60 minutes), and the plate's use is in a positive-working mode only.

US-A-4,405,705 (Etoh et al.) and US-A-4,548,893 (Lee et al.) describe amine-containing polymers for photosensitive materials used in non-thermal processes. The imaged materials also require wet processing after imaging.

Thermal processes using polyamic acids and vinyl polymers with pendant quaternary ammonium groups are described in US-A-4.693,958 (Schwartz et al.), but wet processing is required after imaging. In addition, the polyamic acid switchable polymers in this invention show low discrimination magnitude and the quaternary ammonium-based examples suffer from wash-off problems of both the foreground and the background.

US-A-5,512,418 (Ma) describes the use of polymers having cationic quaternary ammonium groups that are heat-sensitive. However, like most of the materials described in the art, wet processing is required after imaging.

WO 92/09934 (Vogel et al.) describes photosensitive compositions containing a photoacid generator and a polymer with acid labile tetrahydropyranyl or activated ester groups. However, imaging of these compositions converts the imaged areas from hydrophobic to hydrophilic in nature and the imaged areas are prone to scumming.

In addition, EP-A 0 652 483 (Ellis et al.) describes lithographic printing plates imageable using IR lasers, and which do not require wet processing. These plates comprise an imaging layer that becomes more hydrophilic upon imagewise exposure to heat. This coating contains a polymer having pendant groups (such as *t*-alkyl carboxylates) that are capable of reacting under heat or acid to form more polar, hydrophilic groups. Imaging such compositions converts the imaged areas from hydrophobic to relatively more hydrophilic in nature, and thus requires imaging the background of the plate, which is generally a larger area. This can be a problem when imaging to the edge of the printing plate is desired. As with the plates described in WO 92/09934, the plates described in Ellis et al. are also prone to scumming.

Although a number of switchable polymer-based printing plates are known, there remain technical barriers toward the utilization of this technology in commercially feasible products. Three difficulties commonly experienced in the design of switchable polymer-based plates are physical wear of the plates, and the related problems of background scumming and blanket toning.

"Physical wear" refers to the mechanical degradation of a printing plate during the printing process. Sufficient resistance to physical wear is often the major factor in determining whether or not a printing plate will be useful for press runs of very long length.

The problems of scumming (also known as "toning") and blanket toning typically result if ink-rejecting areas of the plate are not sufficiently polar. The uptake of ink in undesired areas of the plate results in the consequent undesirable transfer of ink to the final prints. This manifests itself as an unwanted gray or black color in background areas of the final prints. Scumming may occur in both negative-working plates (in nonimaged areas) and positive plates (in imaged areas). The related problem of blanket toning refers to the buildup of ink in the background areas of the printing press blanket cylinder. Excessive blanket toning results in the necessity of periodically stopping a press run to manually clean the ink from the blanket. This can have a negative impact on the productivity of a printing process.

In conventional developable printing plates, grained, anodized aluminum has proven to be a reliable background substrate. It is mechanically tough and shows little evidence of wear even on very long press runs. The material can also tolerate a wide range of press conditions without showing scumming or excessive blanket toning. Generally, the imaging process imparts a change in solubility to the imaged areas of the plate such that, after wet development, a grained, anodized aluminium surface is selectively exposed. Switchable polymer-based plates, however, are designed such that no portions of the imageable layer of the plate are removed. Thus the favourable background properties of aluminium support substrate cannot be utilized. Not surprisingly, scumming behaviour has been observed in many of the switchable polymer based plates that have been reported in the patent literature.

In EP-A 0 924 102, it is reported that scumming may occur with some known printing plates containing switchable polymers in the imaging layers.

EP 1031 412 describes a heat sensitive lithographic printing plate which can be subjected to aqueous development and can be subjected to recording by a solid laser or semi conductor laser emitting infra red rays. The heat sensitive lithographic printing plate of EP 1031 412 comprises a polymer which is capable of changing its hydrophilicity by heat, and cross linked by a cross linking reaction. The hydrophilicity change is brought about by incorporating groups in the polymer selected from a sulphonic acid ester, sulfonamide group or an alkoxyalkyl ester group.

EP 980 754 discloses a method of making a lithographic printing plate comprising a polymer having at least either a carboxylic acid or carboxylate group capable of causing thermal decarboxylation, and a photopolymer composition for recording by exposure to infra red laser beams. Limited carboxylate groups are disclosed.

US-A-5 910 395 discloses a photosensitive composition comprising an organic backbone, an acidic group on the backbone, a photo curing group, and a photo initiating compound. It is stated that photocuring may take place such that plates coated with the composition can be placed directly on press after exposure with no additional processing steps. Specific types of polymers are disclosed, none of which include quaternary ammonium carboxylate groups on the polymer.

### SUMMARY OF THE INVENTION

The problems noted above are overcome by using a general class of heat-sensitive, switchable polymers that provide a good balance of physical toughness with resistance to scumming and blanket toning when incorporated into an imaging member. The switchable polymers can be obtained by simply reacting any of several carboxylic acid-containing polymers (or polymers containing equivalent groups, such as anhydrides) with a quaternary ammonium hydroxide. In a preferred embodiment, the quaternary ammonium hydroxide contains a substituted -alkylene (C1-C3)-phenyl group. The heat-sensitive polymer, when formulated with a photothermal conversion material and preferably a crosslinking agent, provides a mechanically durable infrared radiation sensitive imaging member that exhibits excellent resistance to scumming and blanket toning.

One embodiment of the present invention is an imaging member comprising a support having thereon a hydrophilic imaging layer comprising a hydrophilic heat-sensitive polymer comprising recurring units that comprise quaternary ammonium carboxylate groups. Preferably, the ammonium carboxylate groups contain at least one substituted -alkylene (C₁-C₃)-phenyl group.

This invention also provides a method of imaging comprising the steps of:
A) providing the imaging member described above, and
B) imagewise exposing the imaging member to energy to provide exposed and unexposed areas in the imaging layer and the imaging member, whereby the exposed areas are rendered more oleophilic than the unexposed areas by heat provided by the imagewise exposing.

In addition, the method of imaging can be extended to be a method of printing by following steps A and B with a further step of
C) in the presence of water or a fountain solution, contacting the imagewise exposed imaging member with a lithographic printing ink, and imagewise transferring the ink to a receiving material.

In a preferred embodiment of this invention, the ammonium ion contains one or more of the following substituents in such a way so as to complete four carbon-nitrogen bonds: substituted or unsubstituted benzyl groups, substituted or unsubstituted phenyl groups, five- or six-membered rings, and indoline or isoindoline rings.

In a particularly preferred embodiment, the ammonium cations used in the heat-sensitive polymers include one or more substituted -alkylene(C₁-C₃)-phenyl groups (preferably benzyl groups), and the result is improved imaging speed and roll-up over many of the heat-sensitive polymers that do not have such groups. The one or more noted alkylenephenyl groups comprise one or more substituents on either or both of the alkylene and phenyl moieties. As described in more detail below, the substitution can be of any of a wide variety of patterns and chemical components.

In another embodiment of this invention, the use of specific ammonium ions alleviates the problem of malodorous emissions. When many common quaternary ammonium carboxylate polymers are subjected to thermal imaging, small molecule amines (such as trimethylamine when the benzyltrimethylammonium cation is used) are given off as reactive byproducts. Many of these amines are malodorous and possibly toxic. This problem has been alleviated using two approaches. The first approach is to utilize spiro-quatemary ammonium cations in which the nitrogen is at the quaternary vertex of the intersecting rings. The second approach is to use specific cations that contain three or four benzyl groups or three or four hydroxyethyl groups.

The imaging member (for example, printing plates) of this invention have improved mechanical durability over other "switchable polymer'' processless printing plates. The imaging member of this invention also exhibits substantially reduced blanket toning and reduced scumming. In some embodiments, the emission of malodorous gases is reduced. In addition, some of the polymers can be prepared easily using very inexpensive materials.

### DETAILED DESCRIPTION OF THE INVENTION

The imaging members of this invention comprise a support and one or more layers thereon that are heat-sensitive. The support can be any self-supporting material including polymeric films, glass, ceramics, metals or stiff papers, or a lamination having a thickness of from 100 to 310 µm. Another preferred embodiment uses aluminum foil having a thickness of from 100 to 600 µm. The support should resist dimensional change under conditions of use.

The support can also be a cylindrical surface having the heat-sensitive polymer composition thereon, and thus being an integral part of the printing press. The use of such imaged cylinders is described for example in US-A-5,713,287 (Gelbart).

The support may be coated with one or more "subbing" layers to improve adhesion of the final assemblage. Examples of subbing layer materials include, but are not limited to, gelatin and other naturally occurring and synthetic hydrophilic colloids and vinyl polymers (such as vinylidene chloride copolymers) known for such purposes in the photographic industry, vinylphosphonic acid polymers, silicon-based sol-gel materials, such as those prepared from alkoxysilanes such as aminopropyltriethoxysilane or glycidoxypropyltriethoxysilane, titanium sol gel materials, epoxy functional polymers, and ceramics.

The backside of the support may be coated with antistatic agents and/or slipping layers or matte layers to improve handling and "feel" of the imaging member.

The imaging members, however, have preferably only one heat-sensitive layer that is required for imaging. This hydrophilic layer includes one or more heat-sensitive polymers, and optionally but preferably a photothermal conversion material (described below), and preferably provides the outer printing surface of the imaging member. Because of the particular polymer(s) used in the imaging layer, the exposed (imaged) areas of the layer are rendered more oleophilic in nature.

The heat-sensitive polymers useful in this invention comprise random recurring units at least some of which comprise quaternary ammonium salts of carboxylic acids. The polymers generally have a molecular weight of at least 3,000 Daltons and preferably of at least 20,000 Daltons.

The polymer randomly comprises one or more types of carboxylate-containing recurring units (or equivalent anhydride units) units identified as "A" below in Structure 1 and optionally one or more other recurring units (non-carboxylated) denoted as "B" in Structure 1.

The carboxylate-containing recurring units are linked directly to the polymer backbone which is derived from the "A" monomers, or are connected by spacer units identified as "X" in Structure 1 below. This spacer unit can be any divalent aliphatic, alicyclic or aromatic group that does not adversely affect the polymer's heat-sensitivity. For example, "X" can be a substituted or unsubstituted alkylene group having 1 to 16 carbon atoms (such as methylene, ethylene, isopropylene, *n*-propylene and *n*-butylene), a substituted or unsubstituted arylene group having 6 to 10 carbon atoms in the arylene ring (such as *m*- or *p*-phenylene and naphthylenes), substituted or unsubstituted combinations of alkylene and arylene groups (such arylenealkylene, arylenealkylenearylene and alkylenearylenealkylene groups), and substituted or unsubstituted N-containing heterocyclic groups. Any of these defined groups can be connected in a chain with one or more amino, carbonamido, oxy, thio, amido, oxycarbonyl, aminocarbonyl, alkoxycarbonyl, alkanoyloxy, alkanoylamino or alkaminocarbonyl groups. Particularly useful "X" spacers contains an ester or amide connected to an alkylene group or arylene group (as defined above), such as when the ester and amide groups are directed bonded to "A".

Additional monomers (non-carboxylate monomers) that provide the recurring units represented by "B" in Structure 1 above include any useful hydrophilic or oleophilic ethylenically unsaturated polymerizable comonomers that may provide desired physical or printing properties of the surface imaging layer or which provide crosslinkable functionalities. One or more "B" monomers may be used to provide these recurring units, including but not limited to, acrylates, methacrylates, styrene and its derivatives, acrylamides, methacrylamides, olefins, vinyl halides, and any monomers (or precursor monomers) that contain carboxy groups (that are not quatemized).

The quaternary ammonium carboxylate-containing polymer may be chosen or derived from a variety of polymers and copolymer classes including, but not necessarily limited to polyamic acids, polyesters, polyamides, polyurethanes, silicones, proteins (such as modified gelatins), polypeptides, and polymers and copolymers based on ethylenically unsaturated polymerizable monomers such as acrylates, methacrylates, acrylamides, methacrylamides, vinyl ethers, vinyl esters, alkyl vinyl ethers, maleic acid/anhydride, itaconic acid/anhydride, styrenics, acrylonitrile, and olefins such as butadiene, isoprene, propylene, and ethylene. A parent carboxylic acid-containing polymer (that is, one reacted to form quaternary ammonium carboxylate groups) may contain more than one type of carboxylic acid-containing monomer. Certain monomers, such as maleic acid/anhydride and itaconic acid/anhydride may contain more than one carboxylic acid unit. Preferably, the parent carboxylic acid-containing polymer is an addition polymer or copolymer containing acrylic acid, methacrylic acid, maleic acid or anhydride, or itaconic acid or anhydride or a conjugate base or hydrolysis product thereof.

In Structure 1, n represents 25 to 100 mol % (preferably from 50 to 100 mol %), and m represents 0 to 75 mol % (preferably from 0 to 50 mol %).

While Structure 1 could be interpreted to show polymers derived from only two ethylenically unsaturated polymerizable monomers, it is intended to include terpolymers and other polymers derived from more than two monomers.

The quaternary ammonium carboxylate groups must be present in the heat-sensitive polymer useful in this invention in such a quantity as to provide a minimum of one mole of the quaternary ammonium carboxylate groups per 1300 g of polymer, and preferably per 1000 g of polymer, and a maximum of one mole of quaternary ammonium carboxylate groups per 45 g of polymer, and preferably per 132 g of polymer. Preferably, this ratio (moles of quaternary ammonium carboxylate groups to grams of polymer) is from 1:600 to 1:132 and more preferably, this ratio is from 1:500 to 1:132, or from 1:500 to 1:45, and more preferably from 1:300 to 1:45. This parameter is readily determined from a knowledge of the molecular formula of a given polymer.

The quaternary ammonium counterion of the carboxylate functionalities may be any ammonium ion in which the nitrogen is covalently bound to a total of four alkyl or aryl substituents as defined below. In a preferred embodiment, at least one of the four substituents is a substituted -alkylene (C₁-C₃)-phenyl group.

More particularly, in Structure 1 noted above, R₁, R₂, R₃ and R₄ are independently substituted or unsubstituted alkyl groups having 1 to 12 carbon atoms [such as methyl, ethyl, *n*-propyl, isopropyl, t-butyl, hexyl, hydroxyethyl, 2-propanonyl, ethoxycarbonymethyl, benzyl, substituted benzyl (such as 4-methoxybenzyl, *o*-bromobenzyl, and *p*-trifluoromethylbenzyl), and cyanoalkyl], or substituted or unsubstituted aryl groups having 6 to 14 carbon atoms in the carbocyclic ring (such as phenyl, naphthyl, xylyl, *p*-methoxyphenyl, *p*-methylphenyl, *m*-methoxyphenyl, *p*-chlorophenyl, *p*-methylthiophenyl, *p*-N,N-dimethylaminophenyl, methoxycarbonylphenyl and cyanophenyl). Alternatively, any two, three or four of R₁, R₂, R₃ and R₄ can be combined to form a ring (or two rings for four substituents) with the quaternary nitrogen atom, the ring having 5 to 14 carbon, oxygen, sulfur and nitrogen atoms in the ring. Such rings include, but are not limited to, morpholine, piperidine, pyrrolidine, carbazole, indoline and isoindoline rings. The nitrogen atom can also be located at the tertiary position of the fused ring. Other useful substituents for these various groups would be readily apparent to one skilled in the art, and any combinations of the expressly described substituents are also contemplated.

At least one of R₁, R₂, R₃ and R₄ is a substituted alkylene (C₁-C₃)-phenyl group. Any two or all three of the remaining substituents may be combined to form a ring or rings as described above.

Preferably, the nitrogen of the quaternary ammonium ion is directly bonded to one or more benzyl groups or one or two phenyl groups. Alternatively, the nitrogen atom is part of one or two five-membered rings, or one or two indoline or isoindoline rings and has a molecular weight of less than 400 Daltons.

The use of a spiro ammonium cation in which the nitrogen lies at the vertex of two intersecting rings is especially preferred. When a carboxylate polymer containing such an ammonium counterion is thermally imaged, small molecule amines are not given off and hence the problem of odor during imaging is alleviated. Similarly, the use of a benzyl-tris-hydroxyethyl ammonium ion may result in the release of triethanolamine that is odorless and relatively benign. This embodiment of the invention is also preferred.

In a preferred embodiment, R₁, R₂ and R₃ are independently linear or branched unsubstituted alkyl groups of 1 to 3 carbon atoms, or linear or branched hydroxyalkyl groups of 1 to 3 carbon atoms that comprise 1 to 3 hydroxy groups as the only substituents (generally only one hydroxy group per carbon atom). More preferably, these radicals are independently methyl, hydroxymethyl, ethyl, 2-hydroxyethyl, 1-hydroxyethyl or 1,2-dihydroxyethyl and most preferably, they are either methyl or 2-hydroxyethyl.

R₄ is preferably a substituted alkylenephenyl group that has at least one substituent on either the alkylene or phenyl moiety of the group. More preferably, the one or more substituents are on the phenyl moiety. The alkylene moiety can be linear or branched in nature and has from 1 to 3 carbon atoms (such as methylene, ethylene, *n*-propylene or isopropylene). Preferably, the alkylene moiety of R₄ has 1 or 2 carbon atoms and more preferably, it is methylene. The alkylene moiety can have as many substituents as there are available hydrogen atoms to be removed from a carbon atom. Useful alkylene substituents are the same as those described below in defining the phenyl substituents, but the most preferred substituents for the alkylene moiety are fluoro and alkoxy.

The phenyl moiety of R₄ can have from 1 to 5 substituents in any useful substitution pattern. Useful substituents include but are not limited to, halo groups (such as fluoro, chloro, bromo, and iodo), substituted or unsubstituted alkyl groups having from 1 to 12 carbon atoms (such as methyl, ethyl, isopropyl, *t*-butyl, *n*-pentyl and *n*-propyl) that can be further substituted with any of the substituents listed herein (such as haloalkyl groups including trihalomethyl groups), substituted or unsubstituted alkoxy groups having 1 to 12 carbon atoms (such as methoxy, ethoxy, isopropoxy, n-pentoxy and *n*-propoxy), cyano, nitro, substituted or unsubstituted aryl groups having 6 to 14 carbon atoms in the aromatic carbocyclic ring (as defined above for R₁, R₂ and R₃), substituted or unsubstituted alkyleneoxycarbonyl groups having 2 to 12 carbon atoms (such as methyleneoxycarbonyl, ethyleneoxycarbonyl and i-propyleneoxycarbonyl), substituted or unsubstituted alkylcarbonyloxy groups having 2 to 12 carbon atoms (such as methylenecarbonyloxy, efhyfenecarbonyloxy and isopropylenecarbonyloxy), substituted or unsubstituted alkylcarbonyl groups having 2 to 12 carbon atoms (such as methoxy, ethoxy, isopropoxy, n-pentoxy, and n-propoxy), cyano, nitro, substituted or unsubstituted aryl groups having 6 to 14 carbon atoms in the aromatic carbocyclic ring (as defined above for R₁, R₂ and R₃), substituted or unsubstituted alkyleneoxycarbonyl groups having 2 to 12 carbon atoms (such as methyleneoxycarbonyl, ethyleneoxycarbonyl and *i*-propyleneoxycarbonyl), substituted or unsubstituted alkylcarbonyloxy groups having 2 to 12 carbon atoms (such as methylenecarbonyloxy, ethylenecarbonyloxy and isopropylenecarbonyloxy), substituted or unsubstituted alkylcarbonyl groups having 2 to 12 carbon atoms (such as methylenecarbonyl, ethylenecarbonyl and isopropylenecarbonyl), amido groups, aminocarbonyl groups, trihalomethyl groups, perfluoroalkyl groups, formyl, mercapto and substituted or unsubstituted heterocyclic groups having 5 to 14 atoms in the ring that includes one or more nitrogen, sulfur, oxygen or selenium atoms with the remainder being carbon atoms (such as pyridyl, oxazolyl, thiphenyl, imidazolyl, and piperidinyl).

Preferably, R₄ contains 1 to 5 substituents (more preferably 1 or 2 substituents) on the phenyl moiety, which substituents are either halo groups, substituted or unsubstituted methyl or ethyl groups, or substituted or unsubstituted methoxy or 2-ethoxy groups. More preferably, R₄ comprises 1 to 3 methyl, fluoro, chloro, bromo or methoxy groups, or any combination of these groups on either the alkylene or phenyl moiety.

The use of the particular ammonium ions in which all of R₁-R₃ are 2-hydroxyethyl groups may result in less odor during imaging the heat-sensitive polymer.

Particularly useful heat-sensitive polymers of these invention are described below as Polymers 11-23 and 25.

The heat-sensitive polymers may be readily prepared using many methods that will be obvious to one skilled in the art. Many quaternary ammonium salts and carboxylic acid or anhydride-containing polymers are commercially available. Others can be readily synthesized using preparative techniques that would be obvious to one skilled in the art. Substituted benzyltrialkylammonium salts can be readily synthesized using preparative techniques that would be obvious to one skilled in the art. One convenient method involves the reaction of a substituted benzylamine with a desired alkyl halide, alkyl sulfonate ester or other alkyl-containing compound having a suitable "leaving" group. Another useful method involves the reaction of a substituted benzylic halide with a trialkylamine.

The carboxylic acid or anhydride-containing polymers can be converted to the desired quaternary ammonium carboxylate salts by a variety of methods including, but not necessarily limited to:
1) the reaction of a carboxylic acid- or acid anhydride-containing polymer with the hydroxide salt of the desired quaternary ammonium ion,
2) the use of ion exchange resin containing the desired quaternary ammonium ion,
3) the addition of the desired ammonium ion to a solution of the carboxylic acid-containing polymer or a salt thereof followed by dialysis,
4) the addition of a volatile acid salt of the desired quaternary ammonium ion (such as an acetate or formate salt) to the carboxylic acid-containing polymer followed by evaporation of the volatile component upon drying,
5) electrochemical ion exchange techniques,
6) the polymerization of monomers containing the desired quaternary ammonium carboxylate units, and
7) the combination of a specific salt of the carboxylic acid-containing polymer and a specific quaternary ammonium salt, both chosen such that the undesired counterions will form an insoluble ionic compound in a chosen solvent and precipitate.

Preferably, the first method is employed.

Although it is especially preferred that all of the carboxylic acid (or latent carboxylic acid) functionalities of the polymer are converted to the desired quaternary ammonium salt, imaging compositions in which the polymer is incompletely converted may still retain satisfactory imageability. Preferably, at least 50 monomer percent of the carboxylic acid (or equivalent anhydride) containing monomers are reacted to form the desired quaternary ammonium groups.

In the preferred embodiments of this invention, the heat-sensitive polymer is crosslinked. Crosslinking can be provided in a number of ways. There are numerous monomers and methods for crosslinking that are familiar to one skilled in the art. Some representative crosslinking strategies include, but are not necessarily limited to:
1) the reaction of Lewis basic units (such as carboxylic acid, carboxylate, amine and thiol units within the polymer with a multifuctional epoxide-containing crosslinker or resin,
2) the reaction of epoxide units within the polymer with multifunctional amines, carboxylic acids, or other multifunctional Lewis basic unit,
3) the irradiative or radical-initiated crosslinking of double bond-containing units such as acrylates, methacrylates, cinnamates, or vinyl groups,
4) the reaction of multivalent metal salts with ligating groups within the polymer (the reaction of zinc salts with carboxylic acid-containing polymers is an example),
5) the use of crosslinkable monomers that react via the Knoevenagel condensation reaction, such as (2-acetoacetoxy)ethyl acrylate and methacrylate,
6) the reaction of amine, thiol, or carboxylic acid groups with a divinyl compound (such as bis(vinylsulfonyl) methane) via a Michael addition reaction,
7) the reaction of carboxylic acid units with crosslinkers containing multiple aziridine or oxazoline units,
8) the reaction of acrylic acid units with a melamine resin,
9) the reaction of diisocyanate crosslinkers with amines, thiols, or alcohols within the polymer,

Ethylenically unsaturated polymerizable monomers having crosslinkable groups (or groups that can serve as attachment points for crosslinking additives) can be copolymerized with the other monomers as noted above. Such monomers include, but are not limited to, 3-(trimethylsilyl)propyl acrylate or methacrylate, cinnamoyl acrylate or methacrylate, N-methoxymethyl methacrylamide, N-aminopropylmethacrylamide hydrochloride, acrylic or methacrylic acid and hydroxyethyl methacrylate.

Preferably, crosslinking is provided by the addition of an epoxy-containing resin to the quaternary ammonium carboxylate polymer or by the reaction of a bisvinylsulfonyl compound with amine containing units (such as N-aminopropylmethacrylamide ) within the polymer. Most preferably, CR-5L (an epoxide resin sold by Esprit Chemicals) is used for this purpose.

The imaging layer of the imaging member can include one or more of such homopolymers or copolymers, with or without up to 50 weight % (based on total dry weight of the layer) of additional binder or polymeric materials that will not adversely affect its imaging properties.

The amount of heat-sensitive polymer(s) used in the imaging layer is generally at least 0.1 g/m², and preferably from 0.1 to 10 g/m² (dry weight). This generally provides an average dry thickness of from 0.1 to 10 µm.

The imaging layer can also include one or more conventional surfactants for coatability or other properties, dyes or colorants to allow visualization of the written image, or any other addenda commonly used in the lithographic art, as long as the concentrations are low enough so they are inert with respect to imaging or printing properties.

Preferably, the heat-sensitive imaging layer also includes one or more photothermal conversion materials to absorb appropriate radiation from an appropriate energy source (such as an IR laser), which radiation is converted into heat. Preferably, the radiation absorbed is in the infrared and near-infrared regions of the electromagnetic spectrum. Such materials can be dyes, pigments, evaporated pigments, semiconductor materials, alloys, metals, metal oxides, metal sulfides or combinations thereof, or a dichroic stack of materials that absorb radiation by virtue of their refractive index and thickness. Borides, carbides, nitrides, carbonitrides, bronze-structured oxides and oxides structurally related to the bronze family but lacking the WO_{2.9} component, are also useful.

One particularly useful pigment is carbon of some form (for example, carbon black). Carbon blacks which are surface-functionalized with solubilizing groups are well known in the art and these types of materials are preferred photothermal conversion materials for this invention. Carbon blacks which are grafted to hydrophilic, nonionic polymers, such as FX-GE-003 (manufactured by Nippon Shokubai), or which are surface-functionalized with anionic groups, such as CAB-O-JET® 200 or CAB-O-JET® 300 (manufactured by the Cabot Corporation) are especially preferred.

Useful absorbing dyes for near infrared diode laser beams are described, for example, in US-A-4,973,572 (DeBoer). Particular dyes of interest are "broad band" dyes, that is those that absorb over a wide band of the spectrum. Mixtures of pigments, dyes, or both, can also be used. Particularly useful infrared radiation absorbing dyes include those illustrated as follows:
IR Dye 1
IR Dye 2 Same as Dye 1 but with chloride as the anion.
IR Dye 3
IR Dye 4
IR Dye 5
IR Dye 6
IR Dye 7
IR Dye 8
IR Dye 9

Useful oxonol compounds that are infrared radiation sensitive include Dye 5 noted above and others described in copending and commonly assigned US 6,423,469-B filed November 22, 1999 by DoMinh et al. and entitled "Thermal Switchable Composition and Imaging Member Containing Oxonol IR Dye and Methods of Imaging and Printing".

The photothermal conversion material(s) are generally present in an amount sufficient to provide an optical density of at least 0.3 (preferably of at least 0.5 and more preferably of at least 1.0) at the operating wavelength of the imaging laser. The particular amount needed for this purpose would be readily apparent to one skilled in the art, depending upon the specific material used.

Alternatively, a photothermal conversion material can be included in a separate layer that is in thermal contact with the heat-sensitive imaging layer. Thus, during imaging, the action of the photothermal conversion material can be transferred to the heat-sensitive polymer layer without the material originally being in the same layer.

The heat-sensitive composition can be applied to the support using any suitable equipment and procedure, such as spin coating, knife coating, gravure coating, dip coating or extrusion hopper coating. The composition can also be applied by spraying onto a suitable support (such as an on-press printing cylinder) as described in US-A-5,713,287 (noted above).

The imaging members of this invention can be of any useful form including, but not limited to, printing plates, printing cylinders, printing sleeves and printing tapes (including flexible printing webs). Preferably, the imaging members are printing plates.

Printing plates can be of any useful size and shape (for example, square or rectangular) having the requisite heat-sensitive imaging layer disposed on a suitable support. Printing cylinders and sleeves are known as rotary printing members having the support and heat-sensitive layer in a cylindrical form. Hollow or solid metal cores can be used as substrates for printing sleeves.

During use, the imaging member of this invention is exposed to a suitable source of energy that generates or provides heat, such as a focused laser beam or a thermoresistive head, in the foreground areas where ink is desired in the printed image, typically from digital information supplied to the imaging device. No additional heating, wet processing, or mechanical or solvent cleaning is needed before the printing operation. A laser used to expose the imaging member of this invention is preferably a diode laser, because of the reliability and low maintenance of diode laser systems, but other lasers such as gas or solid state lasers may also be used. The combination of power, intensity and exposure time for laser imaging would be readily apparent to one skilled in the art. Specifications for lasers that emit in the near-IR region, and suitable imaging configurations and devices are described in US-A-5,339,737 (Lewis et al.). The imaging member is typically sensitized so as to maximize responsiveness at the emitting wavelength of the laser. For dye sensitization, the dye is typically chosen such that its λₘₐₓ closely approximates the wavelength of laser operation.

The imaging apparatus can operate on its own, functioning solely as a platesetter, or it can be incorporated directly into a lithographic printing press. In the latter case, printing may commence immediately after imaging, thereby reducing press set-up time considerably. The imaging apparatus can be configured as a flatbed recorder or as a drum recorder, with the imaging member mounted to the interior or exterior cylindrical surface of the drum.

In the drum configuration, the requisite relative motion between the imaging device (such as a laser beam) and the imaging member can be achieved by rotating the drum (and the imaging member mounted thereon) about its axis, and moving the imaging device parallel to the rotation axis, thereby scanning the imaging member circumferentially so the image "grows" in the axial direction. Alternatively, the thermal energy source can be moved parallel to the drum axis and, after each pass across the imaging member, increment angularly so that the image "grows" circumferentially. In both cases, after a complete scan by the laser beam, an image corresponding to the original document or picture can be applied to the surface of the imaging member.

In the flatbed configuration, the laser beam is drawn across either axis of the imaging member, and is indexed along the other axis after each pass. Obviously, the requisite relative motion can be produced by moving the imaging member rather than the laser beam.

While laser imaging is preferred in the practice of this invention, imaging can be provided by any other means that provides thermal energy in an imagewise fashion. For example, imaging can be accomplished using a thermoresistive head (thermal printing head) in what is known as "thermal printing", described for example in US-A-5,488,025 (Martin et al.). Thermal print heads are commercially available (for example, as Fujitsu Thermal Head FTP-040 MCS001 and TDK Thermal Head F415 HH7-1089).

Without the need for any wet processing after imaging, printing can then be carried out by applying a lithographic ink and fountain solution to the imaging member printing surface, and then transferring the ink to a suitable receiving material (such as cloth, paper, metal, glass or plastic) to provide a desired impression of the image thereon. If desired, an intermediate "blanket" roller can be used to transfer the ink from the imaging member to the receiving material. The imaging members can be cleaned between impressions, if desired, using conventional cleaning means.

The following examples illustrate the practice of the invention, and are not meant to limit it in any way.

**Preparation of Useful Switchable Polymers**

The polymers prepared as described below were characterized as having the ratio of moles of quaternary ammonium carboxylate groups to grams of polymer as shown in TABLE I below.

**TABLE I**

| Polymer | Ratio |
|---|---|
| 1 | 1:221 |
| 2 | 1:235 |
| 3 | 1:230 |
| 4 | 1:311 |
| 5 | 1:207 |
| 6 | 1:245 |
| 7 | 1:293 |
| 8 | 1:245 |
| 9 | 1:228 |
| 10 | 1:221 |
| 11 | 1:235 |
| 12 | 1:249 |
| 13 | 1:251 |
| 14 | 1:256 |
| 15 | 1:300 |
| 16 | 1:239 |
| 17 | 1:251 |
| 18 | 1:235 |
| 19 | 1:291 |
| 20 | 1:263 |
| 21 | 1:290 |
| 22 | 1:290 |
| 23 | 1:311 |
| 24 | 1:311 |
| 25 | 1:325 |

### Preparation of Polymer 1 Solution:

An aqueous solution [60.00 g of a 25% (w/w)] of polyacrylic acid (available from Polysciences, MW ∼ 90,000) was combined with 60.0 g distilled water and 84.63 g of a 41.5% (w/w) methanolic solution of benzyltrimethylammonium hydroxide (Aldrich Chemical). A gummy precipitate initially formed and was slowly redissolved over 30 minutes. The resulting polymer was stored as a 32% (w/w) solution in a water/methanol mixture.

### Preparation of Polymer 2 Solution:

A sample (3.00 g) of polymethacrylic acid (available from Polysciences, MW - 30,000) was combined with 23.00 g of distilled water and 14.04 of a 41.5 % (w/w) methanolic solution of benzyltrimethylammonium hydroxide (Aldrich Chemical). A gummy precipitate initially formed and was slowly redissolved over 30 minutes. The resulting polymer was stored as a 21% (w/w) solution in a water/methanol mixture.

### Preparation of Polymer 3 Solution:

A] A nitrogen-degassed solution of acrylic acid (1.00 g) and 3-aminopropylmethacrylamide hydrochloride (0.13 g) in water (10 ml) were added gradually over one hour using syringe pump to a rapidly stirring, nitrogen degassed solution of 2,2'-azobis(2-methylpropionamidine) dihydrochloride (0.056 g) in water (20 ml) at 60°C. The reaction solution was allowed to stir at 60°C for an additional one hour and was then precipitated into acetonitrile. The solids were collected by vacuum filtration and dried in a vacuum oven at 60°C overnight to afford 0.85 g of the product copolymer as a white powder.
B] A methanolic solution [4.7 ml of a 40 % (w/w)] of benzylltrimethylammonium hydroxide (Aldrich Chemical) was added to a solution of the copolymer from step A (0.85 g) in 8.5 ml of distilled water. A gummy precipitate initially formed and was slowly redissolved over 30 minutes. The solution was diluted with water to a total volume of 23 ml (9.2% solids).

### Preparation of Polymer 4 Solution:

A] Benzyl tris(hydroxyethyl) ammonium bromide (26.78 g, synthesized by the procedure of Rengan et al. (*J. Chem. Soc. Chem. Commun.,* 10*,* 1992, 757) was dissolved in 250 ml of methanol and 5 ml water in a 500 ml round bottomed flask. Silver (I) oxide (20.56 g) was added and the mixture was stirred at room temperature for 72 hours. The insolubles were filtered off and the filtrates were concentrated to 80 ml by rotary evaporation. The clear solution was passed through a flash chromatography column packed with 300 cc³ DOWEX® 550A OH resin using methanol eluent and concentrated to - 50 ml by rotary evaporation. The concentration of hydroxide anion in the solution was determined to be 1.353. meq/g by HCl titration.
B] A 25% (w/w) aqueous solution (12 g) of polyacrylic acid (available from Polysciences, MW - 90,000) was combined with 13.30 g of methanol and 30.75 g of the solution from step A. The resulting polymer was stored as a 25% (w/w) solution in a water/methanol mixture.

### Preparation of Polymer 5 Solution:

An aqueous solution [8.00 g of a 25% (w/w)] of polyacrylic acid (Polysciences, MW ∼ 90,000) was combined with 10.00 g methanol and 12.31 g of a 2.254 meq/g (38.5% w/w) methanolic solution of phenyltrimethylammonium hydroxide (available from TCI America). A gummy precipitate initially formed and was slowly redissolved over 30 minutes. The resulting polymer was stored as a 21 % (w/w) solution in a water/methanol mixture.

### Preparation of Polymer 6 Solution:

A] Pyrrolidine (48.93 g, Aldrich Chemical) was added using an addition funnel over 30 minutes to a solution of α,α'-dibromo-*o*-xylene (45.40 g, Aldrich Chemical) in diethyl ether (408 g). A white precipitate formed almost immediately. The solvent was decanted from the precipitated solid and the crude product was recrystallized from isopropanol, washed three times with diethyl ether, and dried overnight in a vacuum oven at 60°C to afford a very hygroscopic powder. The purified product was stored as a solution in methanol of 25.4% solids.
B] The product solution of step A was combined in a 500 ml round bottomed flask with 9:1 methanol:water (130 ml) and silver (I) oxide (16.59 g). The flask grew slightly warm and the silver (I) oxide turned from black to a dull gray. The reaction solution was allowed to stir for an hour at room temperature and the insolubles were filtered off. The filtrates were passed through a flash chromatography column packed with 300 cm³ of DOWEX® 550A OH resin using a methanol eluent. The collected fractions were concentrated to a weight of 36 g by rotary evaporation. The concentration of hydroxide anion was determined to be 2.218 meq/g by HCl titration.
C] An aqueous solution [12.00 g of a 25% (w/w)] of polyacrylic acid (Polysciences, MW ∼ 90,000) was combined with 11.44 g of methanol and 18.77 g of the solution from step B. A gummy precipitate initially formed and was slowly redissolved over 30 minutes. The resulting polymer was stored as an 18 % (w/w) solution in a water/methanol mixture.

### Preparation of Polymer 7 Solution:

A] Anhydrous ammonia (Aldrich) was bubbled through a rapidly stirring suspension of α,α'-dibromo-*o*-xylene (26.36 g, Aldrich Chemical) in absolute ethanol (300 ml) for 2.5 hours. The reaction mixture was placed in a freezer for 2 hours and then filtered. The collected white solids were washed once with isopropanol and once with diethyl ether to afford 7.95 g of the quaternary ammonium bromide product as fine, white crystals.
B] A sample (7.39 g) of the product from step A was converted from the bromide to the hydroxide using 5.65 g silver (I) oxide and 70 ml of a 9:1 methanol:water mixture in an analogous manner as used for Polymer 6 (Step B). A solution (14.50 g) of 1.452 meq/g of hydroxide anion was obtained.
C] An aqueous solution [5.02 g of a 25% (w/w)] of polyacrylic acid (Polysciences, MW ∼ 90,000) was combined with 14.14 g of methanol and 12.00 g of the solution from step B. A gummy precipitate initially formed and was slowly redissolved over 30 minutes. The resulting polymer was stored as a 16 % (w/w) solution in a water/methanol mixture.

### Preparation of Polymer 8 Solution:

A] Indoline (Aldrich, 14.06 g), 1,4-bromobutane (Aldrich, 25.48 g) and ammonium hydroxide (28% aqueous solution, Aldrich, 45.0 g) were combined in a 500 ml round bottomed flask fitted with an addition funnel and a condenser. The reaction mixture was heated to reflux and 23.0 g of additional ammonium hydroxide solution were added dropwise over 30 minutes. The reaction solution was heated at reflux overnight and the liquids were evaporated from the crude product using a rotary evaporator. The remaining brown solids were dissolved in hot isopropanol and filtered hot to remove residual ammonium bromide. The filtrates were concentrated to an orange oil, dissolved in 200 ml methanol, adsorbed onto 100 cm³ silica gel, and loaded onto the top of a flash chromatography column packed with 1000 cm³ of silica gel. The column was first eluted with 1:1 ethyl acetate:hexane to remove an organic-soluble impurity, and then with methanol to elute the desired product. The collected methanolic solution was concentrated to a yellowish oil on a rotary evaporator to provide 15.0 g of the purified spiro-indolinium bromide salt.
B] All of the purified product from Step A was dissolved in 150 ml of a 9:1 methanol:water mixture. It was then converted to the corresponding hydroxide salt with silver (I) oxide (27.34 g) in an analogous manner as used for Polymer 6 (Step B). A solution (41.9 g) of 1.300 meq/g of hydroxide anion was obtained.
C] A 25% (w/w) aqueous solution (5 g) of polyacrylic acid (Polysciences, MW - 90,000) was combined with 13.34 g of the solution from step B. A gummy precipitate initially formed and was slowly redissolved over 30 minutes. The resulting polymer was stored as a 23.28 % (w/w) solution in a water/methanol mixture.

### Preparation of Polymer 9 Solution:

GANTREZ® AN-139 polymer (ISP Technologies, 1.00 g) was added to a solution comprising distilled water (10 g) and 5.36 g of a 40% (w/w) aqueous solution of benzyltrimethylammonium hydroxide (Aldrich Chemical). The resulting mixture was stirred vigorously for 12 hours at which point a clear, homogeneous solution of 17.80% (w/w) had formed.

### Preparation of Polymer 10 solution:

An aqueous solution (60.00 g, 25% w/w) of polyacrylic acid (Polysciences, MW ∼ 90,000) was combined with distilled water (60 g) and 84.63 g of a 41.5% (w/w) methanolic solution of benzyltrimethylammonium hydroxide (Aldrich). A gummy precipitate initially formed and slowly redissolved over a half-hour. The resulting Polymer 1 was stored as a 32% (w/w) solution in water-methanol. Because this polymer is outside the scope of the present invention (no substituents on benzyl group), this polymer was used to make a Control printing plate.

### Preparation of Solutions of Polymers 11-23:

Polymers 11-23 were all synthesized using a basic three-step process. They are all within the scope of the present invention. The first step involved the reaction of the substituted benzyl halides with 1.5 to 3.0 equivalents of trimethylamine in ether to yield substituted benzyltrimethylammonium halide salts. These salts were characterized by proton NMR and electrospray-MS and the purity was further checked by reverse phase HPLC.

The second step involved the conversion of the halide salts to the corresponding hydroxides using 1.0 equivalents of Ag₂O in methanol-water followed by the removal of volatiles to afford solutions with a hydroxide content of 0.5 to 2.5 mEq/g as determined by HCl titration. The hydroxide salts were characterized by electrospray-MS and the purity was checked by reverse phase HPLC.

The third step was the neutralization of polyacrylic acid (MW = 90,000) with the various substituted benzyltrimethylammonium hydroxides to yield solutions (usually 20% w/w) of the polymers in MeOH/water (having weight ratios ranging from 2:1 to 1:2). A representative procedure is described below for making Polymer 11.

### Preparation of Polymer 11 solution (3 steps):

A] 3-Methylbenzyl bromide (24.64 g, 1.33 x 10⁻¹ mol, Aldrich) was dissolved in 221 g of diethyl ether in a 500 ml round bottomed flask. A 33% (w/w) solution of trimethylamine in methanol (35.80 g, 2.00 x 10⁻¹ mol, Acros) was added all at once, forming a white precipitate almost immediately. The reaction mixture was allowed to stir overnight at room temperature and was then filtered and washed three times with diethyl ether. The resulting white powder was dried in a vacuum oven overnight to afford 29.38 g (90% yield) of 3-methylbenzyl trimethylammonium bromide.
B] The bromide salt from step A (10 g) was dissolved in 100 ml of 9:1 methanol/water in a 250 ml round bottomed flask. Silver (I) oxide (9.5 g, 4.10 x 10⁻¹ mol, Aldrich) was added all at once and stirred for two hours at which point the silver oxide had changed color from a dark black to a dull gray. The solids were then filtered off, first using standard filter paper, then using a 0.5 µm Millipore FC membrane filter. The filtrates were concentrated to a volume of ∼40 ml on a rotary evaporator. The concentration of hydroxide anion in the solution was determined to be 1.237. meq/g by HCl titration.
C] A 25% (w/w) aqueous solution (6.04 g) of polyacrylic acid (Polysciences, MW - 90,000) was combined with 1.79 g methanol and 17.17 g of the solution from step B. A gummy precipitate initially formed and slowly redissolved over a 30 minutes. The polymer was stored as a 20 % (w/w) solution in methanol-water.

Polymers **12-23** were synthesized using analogous procedures. Variations from the representative procedure are noted where applicable in TABLE II below.

### Preparation of Polymer 24 solution (3 steps):

A] Benzyl tris(hydroxyethyl) ammonium bromide was synthesized from triethanolamine and benzyl bromide using the procedure of Rengan et al (*J. Chem. Soc. Chem. Commun.,* 10, 1992, 757).
B] Benzyl tris(hydroxyethyl) ammonium bromide (26.78 g, 8.36 x 10⁻² mol) was dissolved in 250 ml of methanol and 5 ml water in a 500 ml round bottomed flask. Silver (I) oxide (20.56 g, 8.87x10⁻² mol) was added and the mixture was stirred at room temperature for 72 hours. The insoluble materials were filtered off and the filtrates were concentrated to 80 ml by rotary evaporation. The clear solution was passed through a flash chromatography column packed with 300 cm³ DOWEX® 550A OH resin using methanol eluent and concentrated to ∼ 50 ml by rotary evaporation. The concentration of hydroxide anion in the solution was determined to be 1.353. meq/g by HCl titration.
C] A 25% (w/w) aqueous solution (12 g) of polyacrylic acid (available from Polysciences, MW - 90,000) was combined with 13.30 g of methanol and 30.75 g of the solution from step A. The resulting polymer was stored as a 25% (w/w) solution in a water/methanol mixture.

### Preparation of Polymer 25 solution (3 steps):

A] 2-methylbenzyl bromide (10.00g, 5.40x10⁻² mol, Aldrich), triethanolamine (10.48 g, 7.02 x 10⁻² mol, Aldrich), and tetrahydrofuran (54 ml) were combined in a 200 ml round bottomed flask fitted with a reflux condenser and a nitrogen inlet. The reaction was stirred at reflux for 14 hours at which point a large amount of a white solid had formed. The solid was collected by vacuum filtration, recrystallized from ethanol, and dried overnight in a vacuum oven at 60°C. 10.67 g (59% yield) of a fine, white powder was collected.
B] 10.00 g (2.99 x10⁻² mol) of the product from step A was converted to the corresponding hydroxide salt using the procedure described for Polymer 2 (step B). 30 ml of a solution with a hydroxide content of 0.906 mEq/g was obtained.
C] 3.38 g of a 25% (w/w) aqueous solution of polyacrylic acid (available from Polysciences, MW ∼ 90,000) was combined with 1.60 g of methanol and 15.02 g of the solution from step A. The resulting polymer was stored as a 20% (w/w) solution in a water/methanol mixture.

**TABLE II**

| **Polymer #** | **Substituted Benzyl** **halide** | **Step A** **Conditions** | **Step A** **yield** | **[**^{**-**}**OH] (mEq/g) of** **ammonium hydroxide solution** **(Step 13)** |
|---|---|---|---|---|
| 11 | 3-methylbenzyl bromide | Ether, 25°C, 20 hours | 90% | 1.237 |
| 12 | 3,5-dimethylbenzyl bromide | Ether, 25°C, 20 hours | 97% | 1.145 |
| 13 | 1-bromomethyl-3-methoxybenzene | Ether, 25°C, 20 hours | 98% | 1.204 |
| 14 | 3-chlorobenzyl bromide | Ether, 25°C, 20 hours | 98% | 1.256 |
| 15 | 4-bromobenzyl bromide | Ether, 25°C, 20 hours | 99% | 1.330 |
| 16 | 4-fluorobenzyl bromide | Ether, 25°C, 20 hours | 97% | 0.952 |
| 17 | 4-methoxybenzyl chloride | Ether, 25°C, 20 hours | 84% | 2.220 |
| 18 | 4-methylbenzyl bromide | Ether, 25°C, 20 hours | 98% | 1.372 |
| 19 | pentamethylbenzyl chloride | Ether, 3 eq. NMe₃, reflux, 20 hours | 98% | 1.100 |
| 20 | α-chloroisodurene | Ether, 3 eq. NMe₃, 20 hours at 25°C then reflux for 4 hours | 83% | 1.520 |
| 21 | 3,4-dichlorobenzyl chloride | Ether, 3 eq. NMe₃, reflux for 24 hours | 54% | 1.09 |
| 22 | 2,4-dichlorobenzyl chloride | Ether, 3 eq. NMe₃, reflux, 20 hours | 61% | 1.14 |
| 23 | 3,4,5-trimethoxybenzyl bromide* | Ether, 25°C, 20 hours | 88% | 0.516 |

| | | | | |
|---|---|---|---|---|
| *3,4,5-Trimethoxybenzyl bromide was synthesized from 3,4,5-trimethoxybenzyl alcohol using triphenylphosphine/CBr₄. | | | | |

### Example 1: Printing Plate Prepared Using Polymer 1

A coating formulation was prepared comprising Polymer 1 solution (3.74 g), CR-5L (0.12 g, an epoxy resin sold by Esprit Chemicals), FLUORAD® FC-135 cationic surfactant (0.024 g of a 50% solution in isopropanol, 3M Co.), FX-GE-003® (1.80 g, a 10 % dispersion of polymer-grafted carbon black manufactured by Nippon Shokubai), methanol (9.66 g) and water (0.66 g). These components were stirred vigorously in a glass jar for one hour and coated on a mechanically grained and anodized aluminum support at a wet coverage of 2.36 ml/ft² (25.5 ml/m²) that was sufficient to provide a dry coverage of 100 mg/ft² (1.08 g/m²) of polymer, 15 mg/ft² (162 mg/m²) of carbon black, and 10 mg/ft² (108 mg/m²) of CR-5L. The resulting printing plates were dried in an oven at 100 °C for 20 minutes to provide mechanically durable, black imaging layers.

The printing plates were then exposed on a platesetter (similar to the commercially available CREO TRENDSETTER®, but smaller in size) having an array of laser diodes operating at a wavelength of 830 nm each focused to a spot diameter of 23 □m. Each channel provided a maximum of 356 mW of power incident on the recording surface. The printing plates were mounted on a drum whose rotation speed was varied to provide for a series of images set at various exposures as listed in TABLE III below. The laser beams were modulated to produce halftone dot images.

**TABLE III**

| **IMAGE** | **IMAGING POWER** **(mW)** | **IMAGING EXPOSURE** **(mJ/cm**^{**2**}**)** |
|---|---|---|
| 1 | 356 | 360 |
| 2 | 356 | 450 |
| 3 | 356 | 600 |
| 4 | 356 | 900 |

The imaged printing plates were mounted on a commercial A.B. Dick 9870 duplicator press and paper prints were made using VanSon DIAMOND BLACK@ lithographic printing ink and UNIVERSAL PINK® fountain solution containing PAR alcohol substitute (Varn Products Company). It was apparent that the printing plates produced solid images of good quality at the two higher exposure levels. The background showed no scumming and no blanket toning or wear was observed over the press run of 2,000 impressions.

### Example 2: Printing Plate Prepared Using Polymer 2

Printing plates were prepared, imaged, and used for printing as described in Example 1. The imaging layer coating formulation comprised the Polymer 2 solution (5.68 g), CR-5L (0.12 g), FLUORAD® FC-135 cationic surfactant (0.024 g), FX-GE-003 (1.80 g), methanol (8.69 g) and water (8.69 g).

Upon printing, the plates produced solid images of good quality at the two higher exposure levels. The background showed no scumming and no blanket toning or wear was observed over the press run of 2,000 impressions.

### Example 3: Printing Plate Prepared Using Polymer 3

A coating formulation was prepared comprising the Polymer 3 solution (11.04 g), CAB-O-JET® 200 (0.51 g, a 20% dispersion of anionically functionalized carbon black sold by the Cabot Co.), bis(vinylsulfonyl)methane (1.26 g of a 1.8 % solution in water), methanol (5.39 g) and water (1.80 g). The components were combined in a vial and zirconium beads were added to half the height of the vial. This mixture was roll-milled overnight and coated on a gelatin-subbed polyethylene terephthalate support with a wet coverage of 2.36 ml/ft² (25.5 ml/m²) that was sufficient to afford a dry coverage of 100 mg/ft² (1.08 g/m²) of polymer and 10 mg/ft² (108 mg/m²) of carbon black. The printing plates were dried in a convection oven at 80°C for 4 minutes.

The printing plates were then imaged and run on press as described in Example 1. Upon printing, the plates produced solid images of good quality at the highest exposure level. The background showed no scumming and no blanket toning was observed over the press run of 1,000 impressions.

### Example 4: Printing Plate Prepared Using Polymer 4

Printing plates were prepared, imaged and used on press as described in Example 1. The coating formulation comprised the Polymer 4 solution (4.76 g), CR-5L (0.12 g), FLUORAD® FC-135 cationic surfactant (0.024 g), FX-GE-003 (1.80 g), methanol (9.15 g) and water (9.15 g). The imaging exposure series is shown in TABLE IV below.

The printing plates produced solid images of good quality at the higher two exposure levels. The background showed no scumming and no blanket toning or wear was observed over the press run of 2,000 impressions.

**TABLE IV**

| **IMAGE** | **IMAGING POWER** **(mW)** | **IMAGING EXPOSURE** **(mJ/cm**^{**2**}**)** |
|---|---|---|
| 1 | 356 | 602 |
| 2 | 356 | 722 |
| 3 | 356 | 901 |
| 4 | 356 | 1200 |

### Example 5: Printing plate prepared from Polymer 5

Printing plates were prepared as described in Example 1 except that the printing plates were cured at 80°C for 10 minutes. The imaging layer coating formulation comprised the Polymer 5 solution (5.83 g), CR-5L (0.12 g), FLUORAD® FC-135 cationic surfactant (0.024 g), FX-GE-003 (1.80 g), methanol (8.62 g) and water (8.62 g).

The resulting printing plates were imaged in the same manner as described in Example 4 and used for printing in the same manner as described in Example 1. The printing plates produced solid images of good quality at all exposure levels. No wear was observed over the press run of 2000 impressions. To test plate resilience and resistance to scumming, the ink setting on the A.B. Dick duplicator press was maintained at 3 while the fountain solution setting was slowly decreased from 20 (its standard setting) to 12. The background remained very clean until a setting of 14 was reached. As the fountain level was restored to 20, the plates rapidly cleared up and continued to provide good quality impressions.

### Example 6: Printing Plate Prepared Using Polymer 6

Printing plates were prepared as described in Example 1. The imaging layer coating formulation comprised the Polymer 6 solution (6.73 g), CR-5L (0.12 g), FLUORAD® FC-135 cationic surfactant (0.024 g), FX-GE-003 (1.80 g), methanol (8.16 g) and water (8.16 g).

The printing plates were imaged as described in Example 4 and used for printing as described in Example 1. They provided solid images of good quality at the three highest exposure levels. No scumming, blanket toning, or wear was observed over the press run of 2000 impressions.

In another press run, the ink setting on the A.B. Dick duplicator press was maintained at 3 while the fountain setting was slowly decreased from 20 (its standard setting) to 12 in order to test plate resilience and resistance to scumming. The background remained very clean until a setting or 14 was reached. As the fountain level was restored to 20, the printing plates rapidly cleared up and continued to provide good quality impressions.

### Example 7: Printing Plate Prepared Using Polymer 7

Printing plates were prepared as described in Example 1 except that the plate was cured at 80 °C for 20 minutes. The imaging layer coating formulation comprised the Polymer 7 solution (7.30 g), CR-5L (0.12 g), FLUORAD® FC-135 cationic surfactant (0.024 g), FX-GE-003 (1.80 g), methanol (7.88 g) and water (7.88 g).

The printing plates were imaged as described in Example 4 and used for printing as described in Example 1. The printing plates provided solid images of good quality at all exposure levels. No wear was observed over the press run of 2000 impressions. To test plate resilience and resistance to scumming, the ink setting on the A.B. Dick duplicator press was maintained at 3 while the fountain setting was slowly decreased from 20 (its standard setting) to 12. The background remained very clean until a setting or 14 was reached. As the fountain level was restored to 20, the printing plates rapidly cleared up and continued to provide good quality impressions.

### Example 8: Printing Plate Prepared Using Polymer 8

Printing plates were prepared in an identical manner as described in Example 1 except that they were cured at 80°C for 3.5 minutes. The imaging layer coating formulation comprised the Polymer 8 solution (5.12 g), CR-5L (0.12 g), FC-135 (0.024 g), FX-GE-003 (1.80 g), methanol (8.95 g) and water (8.95 g).

The plates were imaged in the same manner as described in Example 4 and run on press in the same manner as described in Example 1. They produced solid images of good quality at all exposure levels. No wear was observed over the press run of 2000 impressions. To test plate resilience and resistance to scumming, the ink setting on the A.B. Dick duplicator press was maintained at 3 while the fountain setting was slowly decreased from 20 (its standard setting) to 12. The background remained very clean until a setting or 14 was reached. As the fountain level was restored to 20, the plates rapidly cleared up and continued to print good quality impressions.

### Example 9: Printing Plate Prepared Using Polymer 9

Printing plates were prepared in an identical manner as described in Example 1 except that they were cured at 80°C for 5 minutes. The imaging layer coating formulation comprised the Polymer 9 solution (6.74 g), CR-5L (0.12 g), FC-135 (0.024 g), FX-GE-003 (1.80 g), methanol (8.16 g) and water (8.16 g).

The plates were imaged in the same manner as described in Example 4 and run on press in the same manner as described in Example 1. They produced solid images of good quality at all exposure levels. No wear was observed over the press run of 2000 impressions.

### Example 10: Printing Plates Prepared Using Polymers 10-25

The formulation, coating, and imaging procedures described herein using polymers 10-25 are analogous to those described hereinabove for polymers 1-9. Coating formulations were prepared using each of the heat-sensitive switchable polymers 10-25 and the additional components in such quantities as to provide 25 g coating mixtures of 6% solids that, when coated at a wet coverage of 2.36 cm³/ft² (25.5 cm³/m²) yield the target dry laydowns listed below in TABLE V. The diluent solvent was either 1:1 methanol:water (Polymers **10-18**) or methanol (Polymers **19-23**). The components were combined in a glass jar and stirred vigorously with a magnetic stirrer for one hour to afford the coating mixtures. The coating mixtures were coated using a digitally controlled syringe drive coating machine on a mechanically grained and anodized aluminum support and dried in an oven at 80°C for 20 minutes.

**TABLE V**

| **Component** | **Laydown (mg/m**^{**2**}**)** |
|---|---|
| Switchable polymer | 1080 |
| CR-5L epoxy resin (Esprit Chemicals) | 108 |
| FC-135 surfactant (3M) | 10.8 |
| FX-GE-003 carbon black dispersion (Nippon Shokubai) | 162 |

### Infrared Exposure and Printing

The printing plates were exposed on an experimental platesetter (similar to the commercially available CREO TRENDSETTER® platesetter, but smaller in size) having an array of laser diodes operating at a wavelength of 830 nm each focused to a spot diameter of 23 µm. Each channel provides a maximum of 450 mW of power incident on the recording surface. The plates were mounted on a drum whose rotation speed was varied to provide for a series of images set at various exposures as listed in TABLE VI below. The laser beams were modulated to produce halftone dot images.

**TABLE VI**

| **Image** | **IMAGING POWER** **(mW)** | **IMAGING EXPOSURE** **(mJ/cm**^{**2**}**)** |
|---|---|---|
| 1 | 356 | 360 |
| 2 | 356 | 450 |
| 3 | 356 | 600 |
| 4 | 356 | 900 |

The exposed printing plates were mounted on a commercial A.B. Dick 9870 duplicator press and prints were made using VanSon Diamond Black® lithographic printing ink and Universal Pink@ fountain solution containing PAR alcohol substitute (Varn Products Company). Each plate was run for 1,000 impressions.

For each plate, the roll-up (number of impressions printed before an image of acceptable density is obtained) and the imaging speed (lowest exposure for which a print of acceptable density was obtained) were noted. The results are tabulated in TABLE VII below. Clearly, all of the Polymers 11-23 showed improvements in both criteria over the Control (Polymer 10) that comprised an unsubstituted benzyl group in the quaternary ammonium cation. Similarly, the 2-methyl substituted N,N,N-tris(hydroxyethyl) ammonium polymer (Polymer **25**) showed notable improvements over Control Polymer 24 that had no substitution on the aromatic ring.

**TABLE VII**

| **Polymer** | **Roll-up** **(number of impressions)** | **Imaging speed** **(mJ/cm**^{**2**}**)** |
|---|---|---|
| **10** (Control) | 200-250 | 900 |
| **11** *m*-methyl substituent | 50 | 450 |
| **12** 2,5-dimethyl substituent | 50 | 450 |
| **13** *m*-methoxy substituent | 100 | 450 |
| **14** *m*-chloro substituent | 50 | 360 |
| **15** *p*-bromo substituent | 75 | 450 |
| **16** *p*-fluoro substituent | 100 | 450 |
| **17** *p*-methoxy substituent | 150 | 600 |
| **18** *p*-methyl substituent | 50 | 450 |
| **19** pentamethyl substituents | 50 | 450-650 |
| **20** 2,4,6-trimethyl substituents | 25 | 450 |
| **21** 3,4-dichloro substituents | 25-50 | 350 |
| **22** 2,4-dichloro substituents | 50 | 450 |
| **23** 3,4,5-trimethoxy substituents | 50-75 | 450-650 |
| **24** tris(hydroxyethyl) Control | 200-250 | 900 |
| **25** tris(hydroxyethyl) (2-methyl substituent) | 50 | 600 |

## Claims

1. An imaging member comprising a support having thereon a hydrophilic imaging layer comprising a hydrophilic heat-sensitive polymer having a backbone and comprising repeating units comprising quaternary ammonium carboxylate groups, wherein the carboxylate groups are linked either directly or indirectly to the polymer backbone, and the quaternary ammonium carboxylate groups comprise at least one substituted -alkylene (C₁-C₃)-phenyl group.

2. The imaging member of claim 1 further comprising a photothermal conversion material.

3. The imaging member of claim 2 wherein said photothermal conversion material is infrared radiation absorbing material and is present in said imaging layer..

4. The imaging member of any one of claims 1 to 3 further comprising a crosslinking agent in said imaging layer.

5. The imaging member of any preceding claim wherein said heat-sensitive polymer comprises at least 1 mole of quaternary ammonium carboxylate groups per 1300g of polymer.

6. The imaging member of any preceding claim wherein said heat-sensitive polymer is represented by Structure 1 below wherein "A" represents recurring units derived from ethylenically unsaturated polymerizable monomers, X is a spacer group, R₁, R₂, R₃, and R₄ are independently alkyl or aryl groups, or any two, three or four of R₁, R₂, R₃, and R₄ can be combined to form one or two heterocyclic rings with the charged nitrogen atom, and B represents non-carboxylated recurring units, m is 0 to 75 mol%, and n is from 25 to 100 mol%, wherein at least one of R₁, R₂, R₃ and R₄ is a substituted-alkylene (C₁-C₃)-phenyl group.

7. The imaging member of claim 6 wherein m is from 0 to 50 mol%, and said B recurring units are derived from at least some additional ethylenically unsaturated polymerizable monomers having unreacted carboxy groups, acid anhydride units or a conjugate base thereof.

8. The imaging member of claim 7 wherein one of said additional monomers is acrylic acid, methacrylic acid, maleic anhydride or a conjugate base or a hydrolysis product thereof.

9. The imaging member of any preceding claim wherein said heat-sensitive polymer is crosslinked with an epoxy-containing resin in said imaging layer.

10. The imaging member of any preceding claim wherein said hydrophilic imaging layer further comprises an epoxy-containing resin to provide crosslinking to said hydrophilic heat-sensitive polymer.

11. The imaging member of claim 6 or 7 wherein m is from 0 to 75 mol%, and said B recurring units are derived from at least some additional ethylenically unsaturated polymerizable monomers having unreacted carboxy groups, acid anhydride groups or a conjugate base thereof.

12. The imaging member of any preceding claim wherein said heat-sensitive polymer comprises spiro-quaternary ammonium cations that are any one of the following cations:

13. A method of imaging comprising the steps of
A) providing the imaging member of any one of claims 1 to 12, and
B) imagewise exposing said imaging member to energy to provide exposed and unexposed areas in the imaging layer of said imaging member, whereby said exposed areas are rendered more oleophilic than said unexposed areas by heat provided by said imagewise exposing.

14. The method of claim 13 wherein said imaging member further comprises a photothermal conversion material, and imagewise exposing is carried out using an IR radiation emitting laser.

15. A method of printing comprising the steps of:
A) providing the imaging member of any one of claims 1 to 12, and
B) imagewise exposing said imaging member to energy to provide exposed and unexposed areas in the imaging layer of said imaging member, whereby said exposed areas are rendered more oleophilic than said unexposed areas by heat provided by said imagewise exposing, and
C) contacting said imagewise exposed imaging member with a fountain solution and a lithographic printing ink, and imagewise transferring said ink to a receiving material.

## Patentansprüche

1. Bildaufzeichnungselement, umfassend einen Träger mit einer darauf befindlichen hydrophilen bilderzeugenden Schicht, umfassend ein hydrophiles wärmeempfindliches Polymer mit einem Grundgerüst und Strukturelementen, die quartäre Ammoniumcarboxylatgruppen umfassen, wobei die Carboxylatgruppen entweder direkt oder indirekt an das Polymergrundgerüst gebunden sind und die quartären Ammoniumcarboxylatgruppen mindestens einen substituierten -Alkylen(C₁-C₃)-phenylrest umfassen.

2. Bildaufzeichnungselement gemäß Anspruch 1, weiterhin umfassend ein photothermisches Umwandlungsmaterial.

3. Bildaufzeichnungselement gemäß Anspruch 2, wobei das photothermische Umwandlungsmaterial ein Infrarotstrahlung absorbierendes Material ist und in der bilderzeugenden Schicht vorhanden ist.

4. Bildaufzeichnungselement gemäß einem der Ansprüche 1 bis 3, weiterhin umfassend ein Vernetzungsmittel in der bilderzeugenden Schicht.

5. Bildaufzeichnungselement gemäß einem der vorstehenden Ansprüche, wobei das wärmeempfindliche Polymer mindestens 1 mol quartäre Ammoniumcarboxylatgruppen auf 1300 g Polymer umfasst.

6. Bildaufzeichnungselement gemäß einem der vorstehenden Ansprüche, wobei das wärmeempfindliche Polymer durch nachstehende Struktur 1 dargestellt ist, wobei "A" von ethylenisch ungesättigten polymerisierbaren Monomeren abgeleitete Strukturelemente bedeutet, X ein Spacerrest ist, R₁, R₂, R₃ und R₄ unabhängig Alkyloder Arylreste sind, oder beliebige zwei, drei oder vier Reste aus R₁, R₂, R₃ und R₄ kombiniert sein können, um einen oder zwei heterocyclische Ringe mit dem geladenen Stickstoffatom zu bilden, und B nicht carboxylierte Struktureinheiten bedeutet, m gleich 0 bis 75 mol-% ist, und n gleich 25 bis 100 mol-% ist, wobei mindestens ein Rest aus R₁, R₂, R₃ und R₄ ein substituierter -Alkylen(C₁-C₃)-phenylrest ist.

7. Bildaufzeichnungselement gemäß Anspruch 6, wobei m gleich 0 bis 50 mol-% ist und die Strukturelemente B von mindestens einigen zusätzlichen ethylenisch ungesättigten polymerisierbaren Monomeren mit nichtumgesetzten Carboxygruppen, Säureanhydrideinheiten oder einer konjugierten Base davon abgeleitet sind.

8. Bildaufzeichnungselement gemäß Anspruch 7, wobei eines der zusätzlichen Monomere Acrylsäure, Methacrylsäure, Maleinsäureanhydrid oder eine konjugierte Base oder ein Hydrolyseprodukt davon ist.

9. Bildaufzeichnungselement gemäß einem der vorstehenden Ansprüche, wobei das wärmeempfindliche Polymer in der bilderzeugenden Schicht mit einem Epoxy enthaltenden Harz vemetzt ist.

10. Bildaufzeichnungselement gemäß einem der vorstehenden Ansprüche, wobei die hydrophile bilderzeugende Schicht weiterhin ein Epoxy enthaltendes Harz umfasst, um die Vernetzung des hydrophilen wärmeempfindlichen Polymers zu ermöglichen.

11. Bildaufzeichnungselement gemäß Anspruch 6 oder 7, wobei m gleich 0 bis 75 mol-% ist, und die Strukturelemente B von mindestens einigen zusätzlichen ethylenisch ungesättigten polymerisierbaren Monomeren mit nichtumgesetzten Carboxygruppen, Säureanhydridgruppen, oder einer konjugierten Base davon abgeleitet sind.

12. Bildaufzeichnungselement gemäß einem der vorstehenden Ansprüche, wobei das wärmeempfindliche Polymer spiroquartäre Ammoniumkationen umfasst, welche beliebige der nachstehenden Kationen sind:

13. Verfahren zur Bilderzeugung, umfassend die Schritte:
A) Bereitstellen eines Bildaufzeichnungselements nach einem der Ansprüche 1 bis 12, und
B) bildweises Aussetzen des Bildaufzeichnungselements einer Energie, um der Energie ausgesetzte und nicht ausgesetzte Bereiche in der bilderzeugenden Schicht des Bildaufzeichnungselements bereitzustellen, wobei die der Energie ausgesetzten Bereiche durch bei dem bildweisen Aussetzen einer Energie bereitgestellte Wärme stärker oleophil gemacht werden als die nicht ausgesetzten Bereiche.

14. Verfahren gemäß Anspruch 13, wobei das Bildaufzeichnungselement weiterhin ein photothermales Umwandlungsmaterial umfasst, und das bildweise Aussetzen einer Energie unter Verwendung eines IR-Strahlen emittierenden Lasers durchgeführt wird.

15. Druckverfahren umfassend die Schritte:
A) Bereitstellen eines Bildaufzeichnungselements nach einem der Ansprüche 1 bis 12, und
B) bildweises Aussetzen des Bildaufzeichnungselements einer Energie, um der Energie ausgesetzte und nicht ausgesetzte Bereiche in der bilderzeugenden Schicht des Bildaufzeichnungselements bereitzustellen, wobei die der Energie ausgesetzten Bereiche durch bei dem bildweisen Aussetzen einer Energie bereitgestellte Wärme stärker oleophil gemacht werden als die nicht ausgesetzten Bereiche, und
C) Kontaktieren des bildweise der Energie ausgesetzten Bildaufzeichnungselements mit einem Feuchtmittel und einer lithografischen Druckfarbe, und bildweises Übertragen der Farbe auf ein Empfangsmaterial.

## Revendications

1. Élément de formation d'image comprenant un support ayant dessus une couche de formation d'image hydrophile comprenant un polymère à commutation thermique hydrophile ayant un squelette et comprenant des motifs répétés comprenant des groupes quaternaires carboxylate d'ammonium, dans lequel les groupes carboxylate sont reliés soit directement soit indirectement au squelette du polymère, et les groupes quaternaires carboxylate d'ammonium comprennent au moins un groupe alkylène en (C₁ à C₃)-phényle substitué.

2. Élément de formation d'image selon la revendication 1, comprenant en outre un matériau de conversion photothermique.

3. Élément de formation d'image selon la revendication 2, dans lequel ledit matériau de conversion photothermique est un matériau absorbant le rayonnement infrarouge et est présent dans ladite couche de formation d'image.

4. Élément de formation d'image selon l'une quelconque des revendications 1 à 3, comprenant en outre un agent de réticulation dans ladite couche de formation d'image.

5. Élément de formation d'image selon l'une quelconque des revendications précédentes, dans lequel ledit polymère à commutation thermique comprend au moins 1 mole des groupes quaternaires carboxylate d'ammonium par 1300 g de polymère.

6. Élément de formation d'image selon l'une quelconque des revendications précédentes, dans lequel ledit polymère à commutation thermique est représenté par la structure 1 ci-dessous, dans laquelle « A » représente des motifs structuraux récurrents provenant de monomères polymérisables éthylèniquement insaturés, « X » est un groupe espaceur, R₁, R₂, R₃ et R₄ sont indépendamment des groupes alkyle ou aryle, ou l'un quelconque des deux, trois, ou quatre de R₁, R₂, R₃ et R₄ peuvent être combinés afin de former un ou deux anneaux hétérocycliques avec l'atome d'azote chargé, et « B » représente des motifs structuraux récurrents non-carboxylés, m est compris entre 0 et 75 mol %, et n est compris entre 25 et 100 mol %, dans laquelle au moins un des groupes R₁, R₂, R₃ et R₄ est un groupe alkylène en (C₁ à C₃)-phényle substitué.

7. Élément de formation d'image selon la revendication 6, dans lequel m est compris entre 0 et 50 mol %, et lesdits motifs structuraux récurrents B proviennent d'au moins certains monomères polymérisables éthylèniquement insaturés supplémentaires ayant des groupes carboxy non polymérisés, des unités d'anhydride acide ou une base conjuguée de ceux-ci.

8. Élément de formation d'image selon la revendication 7, dans lequel un desdits monomères supplémentaires est un acide acrylique, un acide méthacrylique, un anhydride maléique ou une base conjuguée ou un produit d'hydrolyse de ceux-ci.

9. Élément de formation d'image selon l'une quelconque des revendications précédentes, dans lequel ledit polymère à commutation thermique est réticulé avec une résine contenant de l'époxy dans ladite couche de formation d'image.

10. Élément de formation d'image selon l'une quelconque des revendications précédentes, dans lequel ladite couche de formation d'image hydrophile comprend en outre une résine contenant de l'époxy afin de fournir une réticulation audit polymère à commutation thermique hydrophile.

11. Élément de formation d'image selon la revendication 6 ou 7, dans lequel m est compris entre 0 et 75 mol %, et lescits motifs structuraux récurrents B proviennent d'au moins certains monomères polymérisables éthylèn_quement insaturés supplémentaires ayant des groupes carboxy non polymérisés, des groupes anhydride acide ou une base conjuguée de ceux-ci.

12. Élément de formation d'image selon l'une quelconque des revendications précédentes, dans lequel ledit polymère à commutation therm_que comprend des cations spiro-quaternaires d'ammonium, qui sont l'un quelconque des calions suivants :

13. Méthode de formation d'image comprenant les étapes consistant à :
A) fournir l'élément de formation d'image selon l'une quelconque des revendications 1 à 12, et
B) exposer conformément à l'image ledit élément de formation d'image à l'énergie afin de fournir des zones exposées et non-exposées dans la couche de formation d'image dudit élément de formation d'image, par quoi lesdites zones exposées sont rendues plus oléophiles que lesdites zones non-exposées par la chaleur fournie par ladite exposition conformément à l'image.

14. Méthode selon la revendication 13, dans laquelle ledit élément de formation d'image comprend en outre un matériau de conversion photothermique, et l'exposition conformément à l'image est réalisée par le biais d'un laser émettant un rayonnement infrarouge.

15. Méthode d'impression comprenant les étapes consistant à :
A) fournir l'élément de formation d'image selon l'une quelconque des revendications 1 à 12, et
B) exposer conformément à l'image ledit élément de formation d'image à l'énergie afin de fournir des zones exposées et non-exposées dans la couche de formation d'image dudit élément de formation d'image, moyennant quoi les zones exposées sont rendues plus oléophiles que lesdites zones non-exposées par la chaleur fournie par ladite exposition conformément à l'image, et
C) mettre en contact ledit élément de formation d'image exposé à la manière d'une image avec une solution de mouillage et une encre d'impression lithographique, et transférer conformément à l'image ladite encre à un matériau de réception.
